

## UNITED STATES PATENT OFFICE

2,376,210

## ALLOY SUITABLE FOR USE AS A BEARING

Irving R. Valentine, Erie, Pa., assignor to General  
Electric Company, a corporation of New YorkNo Drawing. Application July 22, 1942,  
Serial No. 451,958

6 Claims. (Cl. 75—160)

The present invention is an alloy and more particularly an alloy suitable for use as a bearing. Bearing linings, among other qualifications, must have sufficient hardness to resist effectively deformation due to pounding. A Brinell hardness of about 64.5 is satisfactory and is obtained in bearing alloys which employ a relatively large percentage of tin and a smaller percentage of zinc.

It is an object of the present invention to provide an alloy which is suitable for use as a bearing and which contains neither tin nor zinc. It is a further object of the present invention to provide an efficient bearing alloy which has a suitable degree of hardness and which does not cause scoring or welding in the bearing. Other objects will appear hereinafter.

In carrying my invention into effect, I employ an alloy which consists principally of copper but contains effective quantities of lead, silicon and arsenic. The lead content of the alloy provides some lubrication but its principal use is to reduce the quantity of copper employed. The quantity of lead in the alloy varies from a few per cent up to about 15% by weight of the alloy. A lead content materially greater than 15% will cause sweating of the casting. A preferred range of lead content in the alloy varies from about 10 to about 14%.

The silicon content of the alloy varies from about 1.5 to 3% and provides the necessary degree of hardness in the alloy. The silicon has a tendency to increase the friction of the bearing but this effect is overcome by the presence of arsenic. The arsenic not only overcomes the friction effect of the silicon but eliminates any scoring or welding action in the bearing. The quantity of arsenic employed in general is less than the quantity of silicon in the alloy and varies from about 1 to 2½%. A fraction of a per cent of phosphorus, for example about 20% may be present in the alloy as an impurity without materially impairing the properties of the alloy.

A preferred bearing composition consists of about 12.5% lead, 2.6% silicon, 1.45% arsenic with the balance substantially all copper. This alloy in the as-cast condition has a tensile strength of 33,330 pounds per square inch, a yield point of about 18,850 pounds per square inch, an elongation of 8% in two inches and a Brinell hardness of 71.7. After heat treatment at 500° C. for six hours the following properties are obtained:

|                                          |        |
|------------------------------------------|--------|
| Tensile strength—pounds per square inch— | 36,220 |
| Yield point—do—                          | 20,860 |
| Elongation—per cent in two inches—       | 8.5    |
| Brinell hardness—                        | 76.7   |

When the arsenic and silicon are each above

2% and the ratio of arsenic to silicon is above .80, a slight softening takes place in the alloy.

Silicon bronzes, aluminum bronzes and manganese bronzes when run dry in bearing tests give a high temperature rise in about one minute at a pressure of 300 pounds per square inch and in that period of time weld to the soft steel cylinder cooperating member or score it badly. Although such alloys have the necessary physical properties, for example satisfactory tensile strength, hardness, elongation, etc. they do not stand up when tested as a bearing material. My improved bearing alloy containing arsenic and silicon not only has desirable physical properties but superior qualities as bearing material. For example, various alloy compositions consisting of copper, lead, silicon and arsenic, as hereinbefore set forth, were machined to give a bearing surface of three square inches and were run dry on a soft steel cylinder at a pressure of about 300 pounds per square inch for five minutes. The bearings did not give any indication of welding or scoring. Applicant's preferred alloy composition consisting of about 12.5% lead, 2.6% silicon, 1.45% arsenic with the remainder copper, in the as-cast condition, when operated five minutes showed a maximum temperature of only 230° C. The same alloy after having been heat treated for six hours at 500° C. and when operated five minutes showed a maximum temperature of 218° C.

The properties of the alloy under certain conditions are improved by heat treatment for about four to six hours at temperatures varying from about 400 to about 700° C. If the ratio of arsenic to silicon is within the range of .53 to .80 the heat treatment has advantages particularly with respect to the temperature developed in the bearing under operating conditions. However, when the ratio of arsenic to silicon is materially less than .53 or materially greater than .80 the bearing alloy has more satisfactory temperature properties in the as-cast condition. A heat treatment for about six hours at about 400° C. provides entirely satisfactory results. Heating at higher temperatures as a rule does not materially improve the properties of the alloy.

If desired, manganese may be employed in the alloy although its presence does not result in any outstanding improvement in the alloy. If a small quantity is employed, for example about .75% the alloy has satisfactory properties but a tendency to be somewhat soft in the as-cast and heat-treated condition. If larger quantities are employed, for example up to about 3.75%, the hardness of the alloy in the heat treated condition is satisfactory and considerably greater than the hardness of the alloy in the as-cast condition. The properties of the alloy in general are not improved by the use of manganese.

What I claim as new and desire to secure by Letters Patent of the United States, is:

1. An alloy containing a few per cent but not more than 15% lead, about 1.5 to 3% silicon, about 1% to 2½% arsenic with the remainder substantially all copper.

2. A bearing alloy containing a few per cent and up to about 15% lead, about 1.5 to 3% silicon, about 1 to 2½% arsenic with the remainder substantially all copper.

3. A bearing alloy containing a few per cent and up to about 15% lead, about 1.5 to 3% silicon, about 1 to 2½% arsenic with the remainder substantially all copper, the quantity of arsenic present in the alloy being less than the quantity of silicon.

4. A bearing alloy containing a few per cent and up to about 15% lead, about 1.5 to 3% silicon about 1 to 2½% arsenic with the remainder substantially all copper, the ratio of the arsenic to the silicon being within the range of .53 to .80.

5. An alloy containing about 12.46% lead, about 2.73% silicon, about 1.45% arsenic with the remainder substantially all copper.

6. A bearing alloy containing about 10 to 15% lead, about 1.5 to 3% silicon, about 1 to 2½% arsenic with the remainder substantially all copper.

IRVING R. VALENTINE.